

## UNITED STATES PATENT OFFICE

2,073,977

## MANUFACTURE OF COPPER SULPHATE

Marcel Serciron, Dourdan, France

No Drawing. Application April 4, 1935, Serial  
No. 14,707. In Belgium April 7, 1934

13 Claims. (Cl. 23—125)

The invention relates to the manufacture of copper sulphate.

In prior patent application No. 687,709 dated August 31, 1933 for improvements in the "Manufacture of copper sulphate" of the same applicant, a process has been proposed for manufacturing copper sulphate according to which the attack of the copper is obtained, in the presence of air or oxygen, by means of a compound of chlorine capable of forming chlorine of an oxidizing character, and particularly by means of solutions of hydrochloric acid or of suitable chlorides to which are added substances or compounds adapted to promote the formation of the chlorine of oxidizing character.

As an addition reagent nitric acid was recommended and amongst the solutions to be used for attacking the copper a mixture of hydrochloric and nitric acids was recommended containing about 50 to 80 grams of hydrochloric acid and 5 to 10 grams of nitric acid per litre of the liquor respectively.

It has been found that if copper or a material containing copper is exposed, in the presence of air or oxygen, to the action of a liquor formed with a solution of hydrochloric acid or a suitable chloride in the presence of the ion  $\text{NH}_4^+$ , it is possible to attack and dissolve the copper.

30 The invention therefore consists in causing to act on copper or on a material containing copper, in the presence of air or oxygen, a liquor containing in solution hydrochloric acid or a suitable chloride in the presence of the ion  $\text{NH}_4^+$  for the purpose of attacking and dissolving the copper subsequently to be converted into sulphate.

It has further been found that the attack and the dissolution of the copper may be conveniently obtained if to the liquor containing hydrochloric acid or a suitable chloride, there is added either ammonia or an ammonium salt.

Accordingly the invention also consists in causing to act on copper, or a material containing copper, and in the presence of air or oxygen, a liquor containing in solution hydrochloric acid or a suitable chloride in the presence of the ion  $\text{NH}_4^+$  introduced in the form of ammonia or of an ammonium salt.

50 When the liquor to be used for the attack comprises a solution of hydrochloric acid, good results have been secured when the acid concentration of the liquor is of the order of 70 to 80 grams of chlorine per litre and when the liquor comprises a dissolved chloride, good re-

sults have been obtained with a concentration equivalent to the aforesaid concentration of hydrochloric acid, i. e., from 70 to 80 grams of chlorine per litre.

Thus the invention also consists in attacking the copper or a copper bearing material under the conditions aforesaid, by means of a liquor containing hydrochloric acid with a concentration from 70 to 80 grams of chlorine per litre of the liquor or a suitable chloride with 10 an equivalent concentration.

On the other hand it has been found that if the liquor presents a comparatively high concentration in  $\text{NH}_4^+$  ions, instead of copper sulphate an ammonium-copper sulphate may be 15 obtained in the crystallizing tanks. However such a drawback may be avoided if the concentration of the liquor in  $\text{NH}_4^+$  ions is not over a certain limit, and according to the searches and experiments of the applicant such limit is 20 of the order of 20 grams per litre of the liquor to be used for the attack.

Accordingly the invention also consists in attacking copper or a copper bearing material under the conditions stated in the preceding 25 paragraphs, by means of a liquor containing ammonia or an ammonium salt in such a quantity that the concentration in  $\text{NH}_4^+$  ions of the liquor does not exceed 20 grams per litre.

As already stated the  $\text{NH}_4^+$  ions may be introduced into the liquor by adding ammonia or an ammonium salt therein, and in this latter case the body associated to the ammonia may be chlorine or a chlorine compound, the chlorine so introduced replacing a part of the chlorine content of the liquor due to the presence of the hydrochloric acid or a salt thereof.

Therefore the invention also consists in attacking copper or a copper bearing material, in the presence of air or oxygen, by means of a 40 liquor containing hydrochloric acid or a suitable chloride together with a compound of ammonia with chlorine or a chlorine compound.

When the  $\text{NH}_4^+$  ions are introduced in the liquor in the form of a compound comprising 45 ammonia and chlorine or a chlorine compound, the total concentration of chlorine in the liquor shall not exceed the chlorine concentration of 70 to 80 grams per litre indicated and preferably the concentration of  $\text{NH}_4^+$  ions shall not 50 exceed 20 grams per litre.

Accordingly, the invention further consists in causing copper or a copper bearing material to be attacked, in the presence of air or oxygen, by means of a liquor comprising in solution a 55

compound formed with ammonia and chlorine or a chlorine compound, and in which preferably the concentration in  $\text{NH}_4$  ions does not exceed 20 grams per litre and the chlorine concentration due to the ammonium-chlorine compound or to said compound and an addition of hydrochloric acid or a suitable chloride does not exceed 70 to 80 grams of chlorine per litre.

The copper may be attacked and dissolved in 10 the presence of sulphuric acid, the quantity of which is suitable for the sulphate formation, the liquor loaded with the copper sulphate being carried to the crystallizing tanks in which the copper sulphate is allowed to settle in the usual 15 manner, while the mother liquors, after the concentrations thereof have been restored, are returned to the attack or, alternatively, the copper may be attacked in the absence of sulphuric acid and the copper within the solution converted into 20 sulphate by addition of a suitable quantity of sulphuric acid.

The process may be carried out in any suitable apparatus comprising a tower for the attack including upper and lower chambers separated by a perforated false bottom, pipes issuing into the upper chamber, for introducing the reagents therein, pipes issuing into the lower chamber for supplying air or oxygen to the tower, a pipe leading from the lower part of the 25 tower to the crystallizing tanks and a return pipe for the mother liquors from the crystallizing tanks as well as a pump and fittings to insure the circulation of the liquors between the tower and the crystallizing tanks and eventually the 30 heating of said liquors.

Copper in a divided form such as scraps, hollowshots and the like is introduced within the upper chamber of the tower together with the necessary reagents and air is supplied under 40 pressure to the lower chamber of the tower.

When the attack liquor is sufficiently loaded with copper sulphate, the sulphuric acid having been introduced at the same time as the other reagents, it is allowed to flow to the crystallizing tanks in which the sulphate crystals settle, the settling operation being eventually assisted by lowering the temperature; thereafter the mother liquors are restored in their original concentrations and returned to the upper chamber of the 45 tower to execute the same cycle of operations.

If the sulphuric acid is not introduced in the tower, the liquor from the attack having the copper dissolved therein is allowed to flow into a tank located between the tower and the crystallizing tanks, and in which the sulphuric acid is added in the necessary quantity to form the copper sulphate.

The liquor with the sulphate therein is carried to the crystallizing tanks and after settling of the copper sulphate and addition of the reagents to restore the original concentrations the mother liquors are returned to the tower, for a new cycle of operations.

It is to be understood that the details of the 65 process may be modified according to the circumstances and the material acted upon, the process being carried out either in a continuous or intermittent manner.

I claim:

70 1. A process for manufacturing copper sulphate comprising attacking a copper bearing material, in the presence of an oxygen containing gas by means of a liquor containing in solution chlorine ions and a small quantity of  $\text{NH}_4$  ions with a concentration not exceeding 20 grams per

liter of the liquor thereby causing copper of the copper bearing material to be dissolved, and directly converting the dissolved copper into copper sulphate by means of sulphuric acid.

2. A process for manufacturing copper sulphate comprising attacking a copper bearing material, in the presence of an oxygen containing gas, by means of a liquor containing in solution chlorine ions and a small quantity of  $\text{NH}_4$  ions with a concentration not exceeding 20 grams per 10 liter of the liquor, said  $\text{NH}_4$  ions being introduced into the liquor in the form of ammonia, thereby causing copper of the copper bearing material to be dissolved, and directly converting the dissolved copper into copper sulphate by 15 means of sulphuric acid.

3. A process for manufacturing copper sulphate comprising attacking a copper bearing material, in the presence of an oxygen containing gas, by means of a liquor containing in solution 20 chlorine ions and a small quantity of  $\text{NH}_4$  ions with a concentration not exceeding 20 grams per liter of the liquor, said  $\text{NH}_4$  ions being introduced into the liquor in the form of an ammonium salt, thereby causing copper of the copper bearing 25 material to be dissolved, and directly converting the dissolved copper into copper sulphate by means of sulphuric acid.

4. A process for manufacturing copper sulphate comprising attacking a copper bearing 30 material, in the presence of an oxygen containing gas, by means of a liquor containing in solution chlorine ions and a small quantity of  $\text{NH}_4$  ions with a concentration not exceeding 20 grams per liter of the liquor, the concentration 35 of the chlorine into said solution being of the order of 70 to 80 grams per litre, thereby causing copper of the copper bearing material to be dissolved, and directly converting the dissolved copper into copper sulphate by means of sulphuric 40 acid.

5. A process for manufacturing copper sulphate comprising attacking a copper bearing material, in the presence of an oxygen containing gas, by means of a liquor containing chlorine 45 ions and a small quantity of  $\text{NH}_4$  ions with a concentration not exceeding 20 grams per liter of the liquor, said  $\text{NH}_4$  ions being introduced in the liquor by means of an ammonium chlorine compound, thereby causing copper of the copper 50 bearing material to be dissolved and directly converting the dissolved copper into copper sulphate by means of sulphuric acid.

6. A process in accordance with claim 5, in which the total chlorine concentration does not 55 exceed 70 to 80 grams per litre of the liquor.

7. A process for manufacturing copper sulphate comprising attacking a copper bearing material, in the presence of an oxygen containing 60 gas, by means of a liquor containing in solution chlorine ions and a quantity of  $\text{NH}_4$  ions not exceeding 20 grams per liter of the liquor and adding sulphuric acid to the reaction, whereby the copper is dissolved and directly converted into copper sulphate, and separating 65 the copper sulphate formed.

8. A process for manufacturing copper sulphate comprising attacking a copper bearing material, in the presence of an oxygen containing 70 gas, by means of a liquor containing in solution chlorine ions and a quantity of  $\text{NH}_4$  ions not exceeding 20 grams per liter of the liquor, thereby causing copper of the copper bearing material to be dissolved in the liquor, separating copper containing liquor, adding sul- 75

phuric acid thereto and separating therefrom the copper sulphate formed.

9. A process for manufacturing copper sulphate, comprising attacking a copper bearing material, in the presence of an oxygen containing gas, by means of a liquor containing in solution hydrochloric acid and a small quantity of ammonia the concentration of the  $\text{NH}_4$  ions of the liquor not exceeding 20 grams per liter, thereby causing copper of the copper bearing material to be dissolved, placing said dissolved copper in the presence of sulphuric acid and thus directly converting it into copper sulphate and separating the copper sulphate formed.
10. A process for manufacturing copper sulphate comprising attacking a copper bearing material, in the presence of an oxygen containing gas, by means of a liquor containing in solution hydrochloric acid and a small quantity 15 of ammonia in the form of an ammonium salt the concentration of the  $\text{NH}_4$  ions of the liquor not exceeding 20 grams per liter, thereby causing copper of the copper bearing material to be dissolved, placing said dissolved copper in the presence of sulphuric acid and thus directly 20 converting it into copper sulphate and separating the copper sulphate formed.
11. A process for manufacturing copper sulphate comprising attacking a copper bearing material, in the presence of an oxygen containing 25 gas, by means of a liquor containing in so-

lution a chloride and a small quantity of ammonia the concentration of the  $\text{NH}_4$  ions of the liquor not exceeding 20 grams per liter, thereby causing copper of the copper bearing material to be dissolved, placing said dissolved copper in the presence of sulphuric acid and thus directly converting it into copper sulphate and separating the copper sulphate formed.

12. A process for manufacturing copper sulphate, comprising attacking a copper bearing material, in the presence of an oxygen containing gas, by means of a liquor containing in solution chlorine ions and a quantity of  $\text{NH}_4$  ions not exceeding 20 grams per liter of the liquor and adding sulphuric acid to the reaction, 10 whereby the copper is dissolved and converted into copper sulphate while the  $\text{NH}_4$  content of the liquor remains substantially constant, and separating the copper sulphate formed.

13. A continuous process for manufacturing 15 copper sulphate, comprising attacking a copper bearing material, in the presence of an oxygen containing gas, by means of a liquor containing in solution chlorine ions and a quantity of  $\text{NH}_4$  ions not exceeding 20 grams per liter of the liquor, from time to time adding sulphuric acid 20 to the reaction while the  $\text{NH}_4$  content of the liquor remains substantially constant, and separating out the copper sulphate directly formed 25 in the liquor.

MARCEL SERCIRON.